

Feb. 24, 1959

C. F. SMITH ET AL

2,875,056

POLYSTYRENE PHOTOGRAPHIC ELEMENT HAVING A RESINOUS  
TERPOLYMER CHROMIC CHLORIDE UNDERCOAT

Filed Feb. 14, 1958

Fig. 1



Fig. 2



Fig. 3



CARL F. SMITH  
WALTER R. WHITE  
INVENTORS

BY  
R. Frank Smith  
Leonard E. Branchen

ATTORNEY & AGENT

# United States Patent Office

2,875,056

Patented Feb. 24, 1959

1

2,875,056

## POLYSTYRENE PHOTOGRAPHIC ELEMENT HAVING A RESINOUS TERPOLYMER CHROMIC CHLORIDE UNDERCOAT

Carl F. Smith and Walter R. White, Rochester, N. Y., assignors to Eastman Kodak Company, Rochester, N. Y., a corporation of New Jersey

Application February 14, 1958, Serial No. 715,296

8 Claims. (Cl. 96—87)

This invention relates to polystyrene sheeting and more particularly to an improved oriented polystyrene film base having a resinous undercoat containing a chromium salt and a second coating or overcoat of a mixed gelatin and cellulose nitrate composition, which adhere firmly to the base and each other and permit firm adherence thereto of a further coating thereover of a light-sensitive composition, preferably a gelatino-silver halide emulsion layer, to give a photographic element of greatly improved dimensional stability.

It is known that various synthetic resins adhere to polystyrene sheeting and, accordingly, can be used as subbing compositions over which is coated a light-sensitive gelatin emulsion layer. One of the most satisfactory resins, insofar as adhesion to the polystyrene is concerned, is poly-n-butyl methacrylate. However, a serious drawback to the use of this resinous material is that its softness permits the emulsion layer, under conditions of low humidity, to contract and shrink back from the edge of the film. This defect known as skidding may be eliminated for the most part by hardening the poly-n-butyl methacrylate by incorporating into the coating composition thereof certain harder resins having higher softening points or cellulose nitrate, which are compatible therewith. Too much of the hardening material will, of course, cause separation of the resin subbing layer from the polystyrene sheet. However, even when a proper amount of the harder resins are added to the poly-n-butyl methacrylate, it has been observed that after some time, varying from a few days to a few months, a photographic element using such a subbing layer may show a lifting of the emulsion around the edges of the support or along scribed lines. This is a decided disadvantage in graphic arts and cartographic processes.

We have now found that a greatly improved photographic element that shows firm adherence of the emulsion layer to a polystyrene film base, and more particularly to an oriented polystyrene film base, under the usual conditions of processing and use, may be prepared by using a resinous terpolymer consisting predominantly of n-butyl methacrylate units and lesser amounts of methyl methacrylate and methacrylic acid units in admixture with a chromium salt, and more particularly chromic chloride, in the proportions of from 95—99% of the resinous terpolymer and from 5—1% of the said salt as the undercoat layer. A mixed gelatin-cellulose nitrate overcoat is applied over the undercoat. This combination on photographic elements coated with a gelatino-silver halide emulsion gave photographic elements which showed good adhesion of the layers and the emulsion layer showed no tendency of edge lifting under testing and use conditions.

It is, accordingly, an object of the invention to provide a subbing composition which adheres firmly to polystyrene sheeting, and also firmly anchors light-sensitive gelatin emulsion layers to the subbed sheeting. Another object is to provide an improved photographic element comprising a film base of polystyrene, preferably oriented polystyrene film base, a substratum of the aforesaid sub-

2

bing composition, and a gelatino-silver halide emulsion coated over the subbed surface. Another object is to provide a process for preparing the above subbed sheeting and photographic element. Other objects will become apparent hereinafter.

In accordance with the invention, we prepare the improved photographic element by coating one or both surfaces of oriented polystyrene film base with a subbing composition termed the undercoat, typical compositions coming within the following general formulation given in weight percent:

| Ingredient:                    | Weight percent of total of 100% |
|--------------------------------|---------------------------------|
| Terpolymer                     | 2—6                             |
| 15 50-88% n-butyl methacrylate |                                 |
| 10-40% methyl methacrylate     |                                 |
| 2-10% methacrylic acid         |                                 |
| 20 100%                        |                                 |
| Acetone                        | 15-25                           |
| Isopropyl alcohol              | 70-85                           |
| Chromic chloride               | 0.01-0.60                       |
| Total                          | 100                             |

25 In the above formulation, the proportion of n-butyl methacrylate units in the terpolymer is critical for if the amount is reduced below the lower limit to permit the presence of larger amounts of the harder units, i. e. the methyl methacrylate and methacrylic acid units, poor adhesion to the polystyrene film base will result. On the other hand, if the proportion is increased above the upper limit, adhesion will be improved but skidding of the emulsion layer will become very bad. In the case of the 30 methacrylic acid less than 2% of these units in the terpolymer permits undesired skidding, of the emulsion layer, while above 10% of these units the adhesion to the polystyrene film base begins to decrease sharply. The resinous terpolymer may be prepared by well known polymerization techniques employing the monomers in about the 35 proportions found in the terpolymer, using heat and a peroxide polymerization catalyst. The amount of chromic chloride shown in the formulation is based on the weight of terpolymer used, i. e. 0.5-10%. It is ordinarily added in the form of the hydrate  $\text{CrCl}_3 \cdot 6\text{H}_2\text{O}$  and functions primarily to eliminate dry edge lifting defect. Any amount below or above this range causes poor adhesion between the second coating comprising a mixed 40 gelatin-cellulose nitrate subbing composition and the undercoat.

45 50 After the undercoat has dried, a second subbing composition comprising a mixed gelatin-cellulose nitrate is applied over the above described undercoat layers. Typical compositions of this kind that are useful are those 55 which come within the following general formulation given in weight percent:

| Ingredient:                                          | Weight percent of total of 100% |
|------------------------------------------------------|---------------------------------|
| Gelatin                                              | 0.6-1.75                        |
| Acid dispersing agent for the gelatin                | 0.06-0.15                       |
| Cellulose nitrate                                    | 0.1-0.8                         |
| Acetone                                              | 20-50                           |
| Methyl Cellosolve (ethylene glycol monomethyl ether) | 5-15                            |
| Water                                                | 1-3.5                           |
| Methyl alcohol                                       | 30-75                           |
| Total                                                | 100                             |

70 In the above formulation, the acid dispersing agent may be any of the conventional acids used for dispersing gelatin, e. g. acetic acid. It may vary over a moderately wide range, but preferably about 10% based on the weight of

## 3

the gelatin. The cellulose nitrate is preferably a low viscosity type having a nitrogen content of about 11% and being 80-90% soluble in alcohol. The amount of cellulose nitrate is dependent on the amount of gelatin varying from about 17-46%, based on the weight of the gelatin to give coated layer consisting essentially of from 68-86% by weight of gelatin and 32-14% by weight of cellulose nitrate. The amount of water is also determined on the gelatin content and is present approximately from 2 to 3 times the weight of the gelatin.

When the second subbing layer has dried, an ordinary gelatino-silver halide emulsion is coated thereover and dried. To eliminate any tendency to curl, the other subbed surface is overcoated with a gelatin composition containing no silver halide, but which may contain, if desired, antistatic agents, filter dyes, and the like. The photographic elements produced as above described were characterized by firm adherence of the layers to one another and showed excellent dimensional stability under testing, use and storage conditions.

Representative subbed polystyrene sheeting and photographic elements prepared therewith are shown in cross section in the accompanying drawings illustrating the invention. Referring to the drawings Fig. 1 illustrates an oriented polystyrene film base 10 having a mixed resinous terpolymer and chromic chloride undercoat layer 11 and an overcoat layer 12 of gelatin and cellulose nitrate.

Fig. 2 shows an oriented polystyrene film base 10 having a mixed resinous terpolymer and chromic chloride undercoat 11 on each side and an overcoat of mixed gelatin and cellulose nitrate layer 12 over each undercoat layer 11.

Fig. 3 shows an oriented polystyrene film base 10, having a mixed resinous terpolymer and chromic chloride undercoat layer 11 on each side, an overcoat of mixed gelatin and cellulose nitrate layer 12 over each undercoat layer 11, and a gelatino-silver halide emulsion layer 13 over an overcoat layer 12 and a gelatin layer 14 containing no silver halide over the other overcoat layer 12.

The invention is further illustrated by the following example:

## Example

An oriented polystyrene film base was coated on both sides with the following undercoat composition given in weight percent:

| Ingredient:                                                  | Weight percent of total<br>of 100% |
|--------------------------------------------------------------|------------------------------------|
| Resinous terpolymer                                          | 4                                  |
| 76% n-butyl methacrylate                                     |                                    |
| 19% methacrylate                                             |                                    |
| 5% methacrylic acid                                          |                                    |
| Acetone                                                      | 20                                 |
| Isopropyl alcohol                                            | 75.9                               |
| Chromic chloride (2.5% based on the weight<br>of terpolymer) | 0.1                                |
| Total                                                        | 100                                |

When the undercoatings had dried to give a clear subbed film base, an overcoating composition was applied over the undercoats. It had the following composition given in weight percent:

| Ingredient:                                                                                 | Weight percent of total<br>of 100% |
|---------------------------------------------------------------------------------------------|------------------------------------|
| Gelatin                                                                                     | 1.25                               |
| Acetic acid                                                                                 | 0.15                               |
| Cellulose nitrate (19.3% based on com-<br>bined weight of gelatin and cellulose<br>nitrate) | 0.30                               |
| Acetone                                                                                     | 20.0                               |
| Methyl Cellosolve                                                                           | 10.0                               |
| Water                                                                                       | 2.5                                |
| Methyl alcohol                                                                              | 65.8                               |
| Total                                                                                       | 100                                |

## 4

On drying, a clear subbed film base was obtained. This was then coated with a gelatino-silver halide emulsion on one side, and with a plain aqueous gelatin solution on the other side. The dried photographic film element thus obtained was exposed and processed under standard testing conditions to a negative having sharp definition of the image. It showed no curl on drying and no dry edge lifting even after storage for several months. Scribed lines also were reproduced sharply in the prints made from the scribed negative. Accordingly, the photographic element of this example was found to be a highly satisfactory material for use in graphic arts and cartographic processes.

By following the procedure described in the preceding example, generally similar results were obtained with the other subbing composition of the invention coming within the ranges of ingredients previously set forth. While the subbed styrene sheeting is intended primarily as a base material for the preparation of photographic elements, imbibition blanks, etc. it can also be used for non-sensitized gelatin coatings, e. g. for tapes of various kinds. Such materials may also contain dyes, pigments, and the like for certain desired effects.

What we claim is:

1. A coating composition consisting essentially of from 2-6% by weight of a resinous terpolymer consisting of 50-88% by weight of n-butyl methacrylate units, 10-40% by weight of methyl methacrylate units and 2-10% by weight of methacrylate acid units, 15-25% by weight of acetone, 70-85% by weight of isopropyl alcohol and 0.01-0.60% by weight of chromic chloride.

2. A coating composition consisting essentially of 4% by weight of a resinous terpolymer consisting of 76% by weight of n-butyl methacrylate, 19% by weight of methyl methacrylate and 5% by weight of methacrylic acid, 20% by weight of acetone, 75.9% by weight of isopropyl alcohol and 0.1% by weight of chromic chloride.

3. An oriented polystyrene film base having on at least one side adjacent to said base an undercoat layer consisting essentially of a resinous terpolymer consisting of 50-88% by weight of n-butyl methacrylate units, 10-40% by weight of methyl methacrylate units and 2-10% by weight of methacrylic acid units, and containing 0.5-10.0% of chromic chloride, based on the weight of said terpolymer, and having an overcoat layer directly over at least one of said undercoat layers consisting essentially of 68-86% by weight of gelatin and 32-14% by weight of cellulose nitrate.

4. An oriented polystyrene film base having on at least one side adjacent to said base an undercoat layer consisting essentially of a resinous terpolymer consisting of 76% by weight of n-butyl methacrylate units, 19% by weight of methyl methacrylate units and 5% by weight of methacrylic acid units, and containing 2.5% of chromic chloride based on the weight of the said terpolymer, and having an overcoat layer directly over at least one of said undercoat layers consisting essentially of 80.7% by weight of gelatin and 19.3% by weight of cellulose nitrate.

5. A photographic element comprising an oriented polystyrene film base, an undercoat layer on both sides adjacent to said base consisting essentially of a resinous terpolymer consisting of 50-80% by weight of n-butyl methacrylate units, 10-40% by weight of methyl methacrylate units and 2-10% by weight of methacrylic acid units, and containing 0.5-10.0% by weight of chromic chloride based on the weight of said terpolymer, an overcoat layer directly over each of said undercoat layers consisting essentially of 68-86% by weight of gelatin and 32-14% by weight of cellulose nitrate, a gelatino-silver halide emulsion layer directly over one of said overcoat layers, and a layer consisting essentially of gelatin and devoid of any silver halide directly over the other of said overcoat layers.

6. A photographic element comprising an oriented polystyrene film base, an undercoat layer on both sides adjacent to said base consisting essentially of a resinous terpolymer consisting of 76% by weight of n-butyl methacrylate units, 19% by weight of methyl methacrylate units and 5% by weight of methacrylic acid units, and containing 2.5% of chromic chloride based on the weight of said terpolymer, an overcoat layer directly over each of said undercoat layers consisting essentially of 80.7% by weight of gelatin and 19.3% by weight of cellulose nitrate, a gelatino-silver halide emulsion layer directly over one of said overcoat layers, and a layer consisting essentially of gelatin and devoid of any silver halide directly over the other of said overcoat layers.

7. A process for preparing a photographic element comprising coating an oriented polystyrene film base with an undercoat composition consisting essentially of 2-6% by weight of a resinous terpolymer consisting of 50-80% by weight of n-butyl methacrylate units, 10-40% by weight of methyl methacrylate units and 2-10% by weight of methacrylic acid units, 15-25% by weight of acetone, 70-85% by weight of isopropyl alcohol and 0.01-0.60% by weight of chromic chloride to form undercoat layers adjacent to each side of said base, applying an overcoat composition directly over each of the said undercoat layers consisting essentially of 0.6-1.75% by weight of gelatin, 0.06-0.15% by weight of cellulose nitrate, 0.06-0.15% by weight of an acid dispersing agent for the said gelatin, 20-50% by weight of

acetone, 5-15% by weight of ethylene glycol monomethyl ether, 1-3.5% by weight of water and 30-75% by weight of methyl alcohol to form overcoat layers, and applying a gelatino-silver halide emulsion over one of said overcoated layers, and over the other of said overcoat layers a composition consisting essentially of gelatin and water and being devoid of any silver halide.

8. A process for preparing a photographic element comprising coating an oriented polystyrene film base with an undercoat composition consisting essentially of 4% by weight of a resinous terpolymer consisting of 76% by weight of n-butyl methacrylate units, 19% by weight of methyl methacrylate units and 5% by weight of methacrylic acid units, 20% by weight of acetone, 75.9% by weight of isopropyl alcohol and 0.1% by weight of chromic chloride to form undercoat layers adjacent to each side of said base applying an overcoat composition directly over each of said undercoat layers consisting essentially of 1.25% by weight of gelatin, 0.3% by weight of cellulose nitrate, 0.15% by weight of acetic acid, 20% by weight of acetone, 10% by weight of ethylene glycol monomethyl ether, 2.5% of water and 65.8% by weight of methyl alcohol to form overcoat layers, and applying a gelatino-silver halide emulsion over one of said overcoated layers, and over the other of said overcoat layers a composition consisting essentially of gelatin and water and being devoid of any silver halide.

No references cited.